

J. DAVENPORT.

PROCESS OF UTILIZING THE WASTE PRODUCTS OF GARNET WORKS.  
APPLICATION FILED JAN. 27, 1915.

1,192,394.

Patented July 25, 1916.



Witnesses.

J. Merrill Fuller

William G. Gagen

Inventor.  
John Davenport  
by Heard Smith & Tenant,  
Atty's.

# UNITED STATES PATENT OFFICE.

JOHN DAVENPORT, OF BRIGHTON, MASSACHUSETTS.

## PROCESS OF UTILIZING THE WASTE PRODUCTS OF GARNET-WORKS.

1,192,394.

Specification of Letters Patent. Patented July 25, 1916.

Application filed January 27, 1915. Serial No. 4,763.

*To all whom it may concern:*

Be it known that I, JOHN DAVENPORT, a citizen of the United States, and resident of Brighton, county of Suffolk, State of Massachusetts, have invented an Improvement in Processes of Utilizing the Waste Products of Garnet-Works, of which the following description, in connection with the accompanying drawing, is a specification, like characters on the drawing representing like parts.

The object of this invention is primarily to produce from garnet or from garnet ore an abrasive comprising substantially pure alumina; also to produce therefrom a metal alloy adapted for use in steel manufacture and the like.

A further object of the invention is to utilize the waste products of garnet works such as finely pulverized ore or "garnet flour" in the production of a commercial abradant.

The garnet appears in a variety of forms each of which by reason of its characteristic isometric crystallization, hardness and toughness make it useful in the arts as an abradant, particularly in the manufacture of abrading paper, cloth, belts, etc., for finishing wood, leather and the like.

Garnet, as is well known is found in small quantities in rocks throughout various portions of the United States and elsewhere but usually is commingled with a large proportion of quartz and other minerals which make its commercial extraction prohibitive. In a few places, however, notably in New York State and in New Hampshire, quarries exist which comprise a sufficiently high percentage of almandite crystals cemented together by different amounts of quartz, feldspar, etc., to make its extraction a success commercially. Deposits occur also in Spain and from these three sources the majority, and in fact practically all, of the garnet which is used as an abrasive is obtained.

In the preparation of the abrasive the garnet ore is crushed in the usual manner, screened, and finally separated from the quartz by gravity separation, preferably by means of the Sutton, Steele & Steele concentrating tables or by jigs or it may be

done by means of a magnetic separator. The garnet is then graded and the various grades are then applied by suitable adhesive to paper, cloth, belts or other backing to adapt the same for use in finishing wood and like articles. Because of the cleavage, great hardness, and toughness of the garnet crystals, garnet paper wears much longer than the usual silica coated paper, and in fact does not wear out but merely become filled with fine dust, whereas the crystals of the usual silica papers soon become rounded and worn.

In the preparation of the abradant as above described a considerable quantity of garnet is reduced to a flour of too great fineness to be useful as an abrasive and this material at the present time is wasted. This garnet flour or dust contains a very high percentage of alumina and silica and the purpose of the process herein described is to transform this waste product into valuable products which are useful in the arts.

I have found that by heating the garnet flour above described, or in fact the garnet whether in finely pulverized form or otherwise, in a furnace in the presence of a suitable reducing agent, preferably carbon, two useful products may be obtained, first, practically pure aluminum oxid, *i. e.*, corundum, a well known abradant, and second a ferro-silicon alloy which, as is well known, is useful in the art of steel manufacture.

In the performance of the process herein described any usual form of reducing furnace, preferably an electric furnace may be employed. A convenient form of electric furnace for the purpose is illustrated in section in the accompanying drawing in which the furnace comprises a preferably slightly conical metallic shell 1 which desirably may be made of boiler plate reinforced by hoops or stays 2, suitable rings 3 being secured adjacent to the upper end of the shell to provide means for transporting the shell and for elevating it in case the furnace is to be dismantled. In preparing the furnace for use this shell is placed upon a base 4 of fire brick. A carbon conductor 5 adapted to form one of the electrodes of an electric arc may be embedded in the base 4

and connected in any suitable manner to a cable 6 leading to a preferably alternating current supply of low voltage and high amperage. The shell 1 having been set upon the base 4, a lining of fire bricks 7 is built therein and an inner lining 8 of more refractory bricks such as dolomite, or magnesite formed therein, a layer 9 of the same material being placed on the bricks forming the bottom of the furnace. The top of the furnace desirably comprises a hemispherical dome 10 lined with a highly refractory material 11 such as dolomite or magnesite bricks. The dome 10 is provided with suitable eyebolts 12 preferably secured at equal distances from the center thereof to provide means by which the dome may be readily removed from the furnace. The dome is provided adjacent to the center with an aperture 13 or flue to provide for the escape of the gases formed during the action of the furnace. The opposite side of the dome may be provided with a charging aperture 14 and a suitable cover 15 therefor. The other electrode 16 connected to a cable 17 from the supply is slidably mounted centrally of the dome. This electrode is preferably a carbon cylinder supported by a clamp 18 provided with a rack plate 19 adapted to be engaged by the teeth of a manually or automatically operable gear 20 mounted upon a suitable standard 21 upon the dome.

In the operation of the furnace the electrode 16 is thrust downwardly by rotation of the gear 20 until it contacts with the lower electrode 5. The gear 20 is then rotated in the opposite direction to cause the electrode 16 to move away from the electrode 5 thereby striking the arc. As the charge 22 becomes molten the electrode may be raised gradually to maintain the proper distance between the same and the surface 23 of the molten material.

In the performance of the process with the apparatus above described the furnace is charged with garnet, preferably in the form of dust or flour, intimately mixed with a reducing agent, preferably carbon in the form of coke since it is a good conductor of electricity as well as a desirable reducing agent. The carbon should be added to the garnet in such proportion as to act as a reducing agent upon only those compounds which are to be reduced out of the garnet. Usually eighteen per cent. more or less of carbon by weight is sufficient to add to the charge but this will depend entirely upon the chemical composition of the garnet ore to be treated. When the furnace is charged the upper, movable, electrode 16 is first placed in contact with the lower electrode 5, the current, preferably an alternating current of low voltage and high amperage, turned on and the electrodes separated to

form an arc. The action of the arc rapidly reduces the mixture with which the furnace is charged to a molten state since the pure garnet fuses at the relatively low temperature of about 1260° C. The fusing temperature varies with the amount of ferrous impurities contained therein, being lower in proportion to the greater amount of iron contained in the mixture. Additional material may be introduced until a sufficient amount of molten material is found to be present in the furnace. During the reducing operation an active ebullition occurs, considerable gas being driven off. As the reducing operation proceeds the amount of current is gradually increased until the temperature within the furnace reaches the fusing point of alumina, which is approximately 2050 degrees centigrade. When this temperature is reached it is maintained until the constituents other than alumina are entirely reduced and the ebullition ceases. The current is then slowly cut down, gradually decreasing the temperature to permit the slow crystallization of the alumina.

I have found that when the molten mixture is cooled rapidly it produces a tough glassy substance which is not properly crystallized and does not form a good abrasive, but that when the molten mass is cooled slowly the alumina becomes crystallized throughout. I have also discovered that the ferrosilicon alloy collects in the form of lumps or nodules at the bottom and throughout the mass which may be separated readily from the alumina after the latter is broken.

When the entire mass is cooled sufficiently the furnace may be readily dismantled to permit the mass to be broken up into pieces of suitable size to be crushed in the usual crushers for abrasives. This may be accomplished by lifting off first the dome then the iron shell 1, after which the bricks may be removed to expose the solid mass of alumina. This mass may then be broken by sledges or in any suitable manner and afterward run through the crusher and graded.

The ferrosilicon may be removed from the crushed material in any convenient manner as by a gravity separator of the Sutton, Steele & Steele type and may thereafter be packed for sale to the steel foundries.

I find that by adding silica to the original charge or during the reducing operation aforesaid or by using pulverized garnet ore in which the binder contains silica a higher percentage ferrosilicon may be formed, and that other substances, such as salt ( $NaCl$ ) may be added to the charge to facilitate the fusing and to produce a purer alumina, but ordinarily this is not necessary as the garnet is in itself sufficiently rich in silica and iron for the complete success of the process.

The process above described has been performed mainly upon the variety of garnet known as almandite, mined at Wilmot, N. H., an approximate characteristic chemical analysis of which shows the following:

|                |        |
|----------------|--------|
| Silica         | 36.90  |
| Alumina        | 39.84  |
| Iron oxid      | 18.80  |
| Calcium oxid   | 1.65   |
| Magnesium oxid | 3.27   |
| Manganese oxid | .51    |
|                | 100.97 |

15 This analysis is somewhat inaccurate and high on account of the presence of slight impurities such as biotite, magnetite, quartz, etc., which are always present to a greater or less extent.

20 It is to be understood that other reducing agents than carbon, such as calcium or the like may be used in the performance of this process.

Having thus described my invention, what 25 I claim as new and desire to secure by Letters Patent is;

1. The method of treating garnet which consists in forming a mixture of pulverized garnet with a reducing agent in sufficient 30 amount to reduce the constituents of the garnet other than alumina and insufficient in amount to reduce the alumina, heating the mixture to the fusing temperature of alumina, maintaining said temperature substantially constant until complete fusion of the 35 mass is attained and until the constituents of the garnet other than alumina have been reduced, then gradually reducing the heat supplied and cooling the molten mass slowly 40 to permit crystallization of the alumina and solidification of the products of reduction.

2. The method of salvaging garnet dust or flour to produce artificial alumina and a fer-

rosilicon alloy which consists in mixing in an electric furnace the garnet dust or flour 45 with an amount of pulverized carbon sufficient to reduce the constituents of the garnet other than alumina and insufficient to reduce the alumina, electrically heating the mixture to the fusing temperature of alumina, maintaining said temperature substantially constant until the complete fusion of the mass is attained and the ferrosilicon alloy reduced therefrom, gradually reducing the heat supplied by the electric current and 55 finally cooling the mass slowly to permit complete crystallization of the alumina and the formation of the ferrosilicon alloy into lumps or nodules.

3. The method of producing artificial alumina and its ferrosilicon alloy from garnet consisting in mixing the pulverized garnet with carbon sufficient to reduce the constituents of the garnet other than alumina and insufficient to reduce the alumina, adding to 60 the mixture an amount of silica sufficient to insure the complete reduction of the iron content of the mass to a ferrosilicon alloy, heating the mixture to the fusing temperature of alumina and maintaining the same at 70 such temperature until the ebullition ceases and the reduction of the constituents of the garnet other than alumina is complete, gradually reducing the heat supplied and finally cooling the molten mass slowly to permit the 75 complete crystallization of the alumina and the solidification into lumps or nodules of the ferrosilicon alloy.

In testimony whereof, I have signed my name to this specification, in the presence of 80 two subscribing witnesses.

JOHN DAVENPORT.

Witnesses:

CLARENCE E. JONES,  
THOMAS J. DRUMMOND.